

## UNITED STATES PATENT OFFICE

ROBERT BRACE PENN CRAWFORD, OF CHICAGO, ILLINOIS, AND ROY DIETRICH  
SNYDER, OF HAZLETON, PENNSYLVANIA

## ELECTROPLATING PROCESS

No Drawing. Application filed November 26, 1921, Serial No. 517,895. Renewed January 23, 1930.

The present invention relates to an improved electroplating process whereby non-ferrous metals, for example, an alloy of copper and nickel, are deposited on a base of 5 metal, or other suitable material.

A particular object of this invention is to form a coating or skin for metals of a nickel-copper alloy that possesses all the advantages of the pure nickel coating, but which is less 10 expensive to produce, and, due to its non-corrosive qualities forms a protective and lustrous homogeneous deposit on metal articles, such as pipes, conduits, valves, etc., that otherwise when subjected to the tarnishing influence 15 of the atmosphere and the corrosive effects of liquids, would deteriorate. The alloy deposit has properties resembling "Monel" metal.

The electrolytic bath employed for depositing the alloy upon non-ferrous metals is composed of the following ingredients in substantially the proportions herein set forth:

Nickel sulfate ( $\text{NiSO}_4 \cdot 6\text{H}_2\text{O}$ ), 80 oz. (600 g. per liter). Copper acetate ( $\text{Cu}(\text{Ac})_2$ ),  $2\frac{2}{3}$  oz. (20 g. per liter). Nickel acetate ( $\text{NiAc}_2$ ),  $5\frac{1}{3}$  oz. (40 g. per liter). Sodium chloride ( $\text{NaCl}$ ),  $1\frac{1}{3}$  oz. (10 g. per liter).

The above named ingredients are mixed in about a gallon of water with one part in 2000 30 of white glue, or any other kind of glue, for example commercial liquid glue, the purpose of which is to act as an addition agent. The bath at ordinary room temperature has passed through it an electric current of approximately 35 ly 2 amperes per square foot density on the cathode, and is allowed to age for about four hours.

The length of time that the current may pass will vary, dependent on the thickness of 40 the deposit desired. In practicing the invention, current has been passed for about thirty (30) minutes on an average, giving a relatively thin plate which, while it would take a polish, would not be heavy enough for a protective coating. In applying protective coatings for which heavier plates are desired, we have run the current for three (3) or four (4) hours. Within certain limits it is immaterial for any given weight of plate whether 45 you use high current density, for short pe-

riods, or whether you run for a long time at a low current density. For instance, at a current density of  $0.5 \text{ amp}/\text{dm}^2$  we get a deposit of .03 of a gram of copper nickel alloy on a 30 sq. cm. Platinum foil in thirty (30) minutes. 55 On the same foil, at a current density of 2.0 amperes per square decimeter, we get .17 gm. deposit of copper nickel alloy in thirty (30) minutes. At a current density of  $1.0 \text{ amps}/\text{dm}^2$  we get .18 gm. of copper nickel alloy deposited in one hour on the same electrode. 60

For plating iron and steel, the bath will be compounded of the following ingredients, mixed in about a gallon of water:

Nickel ammonium sulfate

$(\text{NiSO}_4(\text{NH}_4)_2\text{SO}_4 \cdot 6\text{H}_2\text{O})$ ,

13 oz. (97.5 g. per liter). Copper oxalate ( $\text{CuC}_2\text{O}_4$ )  $\frac{1}{2}$  oz. (3.75 g. per liter). Boric acid 70 ( $\text{H}_3\text{BO}_3$ ),  $2\frac{2}{3}$  oz. (20 g. per liter). Nickel chloride ( $\text{NiCl}_2$ ), 1 oz. (7.5 g. per liter), and enough ammonium hydroxide ( $\text{NH}_4\text{OH}$ ) to dissolve the copper oxalate. In some cases we may add about one part in 2000 of glue, as 75 stated above.

This bath has passed through it an electric current of approximately five amperes per square foot density on the cathode, and is allowed to age for about four hours. As hereinbefore stated, the length of time that the current is allowed to pass will depend on the thickness of the plate or coating desired.

While we have selected copper salts of organic acids for use in the electrolytes; we do 85 not wish to be limited thereby, as salts of other acids are operative.

The object to be coated or plated in these baths form the cathode or negative electrode, while the copper-nickel alloy forms the anode 90 or positive electrode. Several anodes may be used. The object to be coated is slowly drawn through the bath between the copper-nickel alloy, that is, the anodes. Standard types of electroplating machines may also be used. 95 The percentage of the copper deposit on the metal will, of course, be affected by the composition of the bath, the temperature, the degree of agitation, and current density.

The composition of the bath, the temper- 100

ature, the degree of agitation and the current density all affect the percentage of copper in the deposit. By aging the solution for several hours under a given set of conditions, the composition of the bath so varies that the percentage of copper in the plate is the same as the percentage of copper in the anode. Hence, by suitable investigation corresponding equilibrium values for concentration, current density, agitation and temperature can be determined in advance and the time of aging reduced.

The character of the deposit from any given bath is influenced only by the acidity or basicity of the solution. If the current efficiency is greater at the anode than at the cathode, the solution grows basic, and this effect can be obviated by allowing the dilute sulfuric or acetic acid to flow in the agitated electrolyte drop by drop at a calibrated rate to keep the acidity (hydrogen-ion concentration) constant or "normal". If the current efficiency at the cathode is higher than at the anode, the solution grows acid. To remedy this, the solution is preferably drawn off from the top and filtered through a predetermined mixture of copper and nickel hydroxid, thereby dissolving some of the hydroxids, and returned to the electrolyte thus keeping the hydrogen-ion concentration constant. As all alloys have different anodic current efficiencies, no specific directions can be given. Cast alloys have higher efficiencies as anodes than rolled or cold worked ones. The anodic current efficiency can be varied by the addition of chlorides to the bath, for example, nickel chloride, or sodium chloride, although more than one and one-third ounces per gallon effects the quality of the deposit.

40 A desired mixture of copper and nickel hydroxids may be obtained by adding an excess of sodium hydroxid to a satisfactorily mixed and aged "normal" electrolyte, and boiling until the ammonia fumes are expelled. The precipitate is filtered and washed. The mixture may also be obtained by precipitating any desired solution of copper and nickel salts.

For commercial operation the balancing of 50 anodic and cathodic current efficiencies is superior to the corrections for acidity or basicity mentioned above. This balancing can easily be accomplished by the following method: Choose the copper nickel alloy it is desired to plate; use cast anodes of this alloy if commercially practicable; add enough chloride to make the average anodic current efficiency equal to the average cathodic efficiency. Usually sodium chloride is added, although nickel chloride is preferable in many instances.

The iron present in many copper-nickel alloys does not materially interfere with the effective operation of the bath, but it can be 60 removed by circulating the electrolyte

through a precipitating bath, adding basic nickel carbonate and filtering, if its presence impairs the quality of the deposit on the metal.

It is to be understood that the proportions 70 of the ingredients above set forth may be varied to a considerable extent and still be within the scope of the present invention.

We claim:

1. An electrolyte for electrodepositing an 75 alloy of copper and nickel, which comprises nickel ammonium sulfate, copper oxalate, boric acid, nickel chloride, ammonium hydroxid, and water.

2. The method of electrodepositing a copper-nickel alloy upon a cathode, which comprises passing an electric current from anodes containing copper and nickel, to a cathode, through an electrolyte containing a nickel salt composed of one of a group comprising 80 sulphates, acetates and chlorides, a copper salt of an acid which dissociates very slightly, a soluble chloride, and water.

3. The method of electrodepositing a copper-nickel alloy upon a cathode, which comprises passing an electric current from an anode containing copper and nickel to a cathode, through an electrolyte containing a nickel salt composed of one of a group comprising 85 sulphates, acetates and chlorides and a copper salt of an acid group, comprising acetates and oxalates, and aging the solution with an anode having the composition 90 it is desired to deposit.

4. The method of electrodepositing a copper-nickel alloy upon a cathode, which comprises passing an electric current from an anode containing copper and nickel to a cathode through an electrolyte containing a nickel salt composed of one of a group comprising 100 sulphates, acetates and chlorides and a copper salt of the acid group, comprising oxalates and acetates, and maintaining the neutral condition of the electrolyte by 105 correcting its acidity during use.

5. An electrolyte for electrodepositing an alloy of copper and nickel, which comprises a nickel salt composed of one of a group comprising sulphates, acetates and chlorides, a copper salt of a group including acetates and oxalates, a soluble chloride and water. 115

6. An electrolyte for electrodepositing an alloy of copper and nickel, which comprises a nickel salt composed of one of a group comprising sulphates, acetates and chlorides, a copper salt of a group including acetates and oxalates, a soluble chloride, ammonium hydroxid and water. 120

7. An electrolyte for electrodepositing an alloy of copper and nickel, which comprises a nickel salt composed of one of a group comprising sulphates, acetates and chlorides, a copper salt of a group including acetates and oxalates, a soluble chloride, ammonium hydroxid, boric acid and water. 125

8. An electrolyte for electrodepositing an alloy of copper and nickel, which comprises a nickel salt composed of one of a group comprising sulphates, acetates and chlorides, a copper salt of a group including acetates and oxalates, a soluble chloride, ammonium hydroxid, boric acid, glue and water.

9. An electrolyte for electrodepositing an alloy of copper and nickel, which comprises 10 two nickel salts from a group comprising sulphates, acetates and chlorides, one of such salts being in excess of the other, a copper salt of an acid group comprising oxalates and acetates, a soluble chloride and water.

15 10. An electrolyte for electrodepositing an alloy of copper and nickel, which comprises a nickel sulphate and a nickel salt from a group comprising chlorides and acetates, a copper salt of an acid group comprising oxalates and acetates, a soluble chloride and water.

11. An electrolyte for electrodepositing an alloy of copper and nickel, which comprises ammonium sulphate, nickel chloride, a copper salt of the acid group comprising oxalates and acetates, boric acid, ammonium hydroxid and water.

12. An electrolyte for electrodepositing an alloy of copper and nickel, which comprises 30 a nickel sulphate, a nickel salt of a group comprising chlorides and acetates, copper acetate, sodium chloride, glue and water.

In testimony whereof we have hereunto set our hands.

35 ROBERT BRACE PENN CRAWFORD.  
ROY DIETRICH SNYDER.

40

45

50

55

60

65